# EUROPEAN PATENT APPLICATION

(11) **EP 0 202 799 A2**
(43) Date of publication of application: **26.11.1986**
(21) Application number: 86303276.9
(22) Date of filing: 30.04.1986
(51) Int. Cl.: B22D 25/00, B22D 19/06

(54) **Method of making a hollow working tool**

(30) Priority: 14.05.1985 GB 8512168
(71) Applicant: Vickers Shipbuilding & Engineering Limited, Barrow-in-Furness Cumbria LA14 1AF (GB)
(72) Inventor: Alldread, Michael David, Barrow-in-Furness Cumbria LA14 4HE (GB)
(74) Representative: Orr, William McLean

(57) **Abstract**

A method of making a hollow working tool for the treatment of a predetermined shaped portion of a workpiece, and particularly a hollow inductor for use in inductive heat treatment of a workpiece. The method comprises casting a solid blank (B) which has an external profile which corresponds with the required external profile of the inductor (1) e.g. the tooth space (11) between two adjacent gear teeth - (10), the blank being made of an electrically conductive material having a relatively low melting point and and being (a) cast in a shape having an external profile which is undersized in a predetermined manner relative to the required external profile of the inductor or (b) subsequently reduced in size so as to provide this undersized external profile. A thick metallic coating is applied to the undersized external profile of the blank so as to provide a composite structure having an external profile which corresponds with the required external profile of the inductor (or which is worked subsequently to provide this profile).

the coating is made of a material having a significantly higher melting point than that of the cast material forming the blank, and is of sufficient thickness to provide a rigiod structure upon subsequent removal, by heating, of the material forming the cast blank.

## Description

This invention relates to a method of making a hollow working tool for the treatment of a predetermined shaped portion of a workpiece, the tool having a predetermined external profile which corresponds generally with the shaped portion of the workpiece which is to be treated by the working tool.

the present invention has been developed primarily, though not exclusively, in relation to the manufacture of a hollow inductor for use in an induction hardening machine.

Current methods of making an inductor for use in an induction hardening machine involve fabrication of the component parts of the inductor by skilled craftsmen, and this imposes significant labour costs, and also means that very painstaking work is involved. Accordingly, there exists a need to provide a simpler method of making inductors involving lower tabour costs, and yet providing easily reproducible manufacture to suit particular workpieces which are to be subjected to inductive hardening.

Inductors are used for hardening workpieces made of metals and metal alloys. In this specification, the term "inductor" is used to define an actual element, through which electrical current passes, and a magnetic intensifier incorporated in the inductor, to cause eddy currents to be induced in the adjacent metal of the workpiece.

The method of this invention is particularly suitable for making inductors to be used for the hardening of gear teeth, though it should be understood that the method has many other applications for making hollow working tools for the treatment of a predetermined shaped portion of a workpiece, in which the tool is formed with a predetermined external profile which corresponds generally with the shaped portion of the workpiece which is to be treated by the working tool. In addition, the method has applciation in the manufacture of hollow conductors of intricate construction and closely toleranced dimensions, when required.

In our co-pending patent applciation No. 8417700 (published specification GB 2 143 854A), there is disclosed a method and apparatus for induction hardening of gear wheels. An induction hardening machine is provided which includes an inductor which is caused to traverse along the gap defined between an adjacent pair of gear teeth of a gear in order to carry out induction hardening. The process is carried out according to a carefully controlled set of operating parameters, in order to achieve the formation of a surface-hardened layer along the working surfaces of the gear teeth, which provides enhanced operating performance of the gear wheel so as to be able to operate satisfactorily for prolonged periods of time under arduous loading conditions. One of the crucial parameters in a successful operation of the process concerns the size and positioning of the inductor within the gear tooth space.

Referring now to Figures 1 to 3 of the accompanying drawings, there is shown schematically an inductor for use in an induction hardening machine, of the general type which is disclosed in more detail in GB specification No. 2 143 854A to which attention is drawn. Figure 1 is a perspective view of the inductor and a connector block assembly for mounting in an induction heating head. Figure 2 is a perspective view of the inductor during fabrication, but before a magnetic intensifier has been fitted therein. Figure 3 is a sectional elevation showing the arrangement of the inductor as it traverses along the gear tooth space, and also shows the clearances at the root and along the flanks of the adjacent gear teeth which define the gear tooth space.

Referring now to Figure 1, this shows an inductor which comprises a copper fabrication 1 enclosing a magnetic intensifier 2. The inductor is supported via copper pipes 4 from connector blocks 5, which may be secured to the induction heating head (not shown) of the apparatus. The size of the inductor will be determined by the tooth gap space defined between a pair of adjacent teeth of a gear wheel which is to receive induction hardening, and necessarily the inductor 1 will be of a relatively small size. However, the inductor is shown in an enlarged perspective view in Figure 2, which illustrates the complexity of the copper fabrication 1, which obviously gives rise to considerable manufacturing difficulties of assembly for the actual size (smaller) of the inductor than that shown in Figure 2. The inductor basically comprises two hollow triangular end sections 6 whciha re connected at their apices by a conduit 7. Annealed copper plate is used for the manufacture, as copper is the preferred material of construction in order to conduct the high level of alternating current required for induction heating. The entire fabrication is hollow so that the cooling water can pass down one pipe 8, via one end section 6, apical conduit 7, second end section 6 and out via the second copper pipe 8. As the hardening operation is conducted under mineral oil for particular reasons, including heat transfer and rate of cooling, the leakage of cooling water from the inductor cannot be tolerated. As disclosed in more detail in GB Specification No. 2 143 854A for satisfactory induction hardening it is essential to carefully control a number of different operating parameters, including particularly control over the clearances between the external profile of the inductor and the adjacent surfaces of the gear tooth flanks and root. Referring now to Figure 3, this shows a clearance which is approximately constant around the root, i. e. A' to A'. Thereafter, from A to B, the clearance between the inductor side and the gear flank progressively increases. Moreover, the centre line of the inductor is located as near to the centre line of the gear tooth space as possible.

After fabrication of the inductor (copper fabrication 1 and magnetic intensifier 2), the sides and apex are carefully profiled to achieve the required clearances, as shown in Figure 3.

A person skilled in the art will readily appreciate the level of skill required to make an inductor, as shown in Figures 1 to 3, by fabrication, and also the time consumed in the manufacture. As a new inductor is required for each new gear tooth profile and size of gear tooth space, the time (and hence cost) of manufacture is a significant on-cost to the commercial exploitation of the induction hardening process which is disclosed in our GB specification No. 2 143 854A. In order to enhance the technical and commercial advantages of the process and apparatus disclosed in our GB specification No. 2 143 854A, it would be advantageous to provide a cheaper method having at least the same accuracy of manufacture of the inductor, as the previously employed manual fabrication techniques. Furthermore, the existing techniques necessarily have a lower limit to the size of inductor which can be made to the required accuracy, and hence gears below a certain physical size cannot currently be induction hardened with currently available inductors, using the process and apparatus disclosed in our GB specification No. 2 143 854A.

As indicated above, the present invention has been developed primarily with a view to providing an improved method of manufacture of an inductor for use in an induction hardening method and apparatus, though the invention is not limited to manufacture of such hollow working tools, and has application to the manufacture of other hollow working tools in which it is necessary to provide a carefully controlled predetermined external profile.

According to one aspect of the invention there is provided a method of making a hollow working tool for the treatment of a predetermined shaped portion of a workpiece, the tool having a predetermined external profile which corresponds generally with the shaped portion of the workpiece which is to be treated by the working tool, and the method comprising:
casting a solid blank which has an external profile which corresponds generally with the required extern_al profile of the tool, the blank being (a) cast in a shape having an external profile which is undersized in a predetermined manner relative to the required external profile of the tool or (b) subsequently reduced in size so as to provide this undersized external profile;
applying a thick metallic coating to the undersized external profile of the blank so as to provide a composite structure having an external profile which corresponds, or which is subsequently worked so as to correspond with the required external profile of the tool, the coating being of sufficient thickness to provide a rigid structure upon subsequent removal of the material forming the cast blank ; and
removing the cast material from the composite structure, thereby forming the hollow working tool with the required external profile.

Preferably, the coating is made of a material having a significantly higher melting point than that of the cast solid blank, and the cast material is removed from the composite structure by the application of sufficient heat to melt the cast material, which may then be poured out of the composite structure. However, it is not essential for the coating to have much higher melting point than the case material and other means than the application of heat material and other means than the application of heat may be employed in order to remove the cast material e.g. chemical means, which selectively dissolve the cast material and leaves the thick coating substantially intact.

It is preferred that the thick metallic coating is applied by electrodeposition, in which case conveniently the cast material which forms the blank is metallic. However, electrodeposition is not the only means which may be adopted to form the thick metallic coating. Furthermore, when the coating is formed by electrodeposition, the cast material does not have to be metallic, as other materials, such as specialised electrically conductive plastics materials, may be used as the core on which the electrodeposition of the metallic coating takes place. In addition, the cast material may even be non-conductive, provided that a conductive film is applied onto its external surface in order to promote electrodeposition of the coating thereon.

The method according to the invention is particularly, though not exclusively, suitable for making a hollow workign tool in the form of a hollow inductor for use in an induction hardening machine.

Therefore, according to a further aspect of the invention, there is provided a method of making a hollow inductor for use in inductive heat treatment of a predetermined shaped portion of a workpiece, by traversing the inductor along the surface of the shaped portion, the inductor having an external profile which corresponds generally with the shaped portion of the workpiece, and the method comprising:
casting a solid blank which has an external profile which corresponds generally with the required external profile of the inductor, the blank being made of an electrically conductive material having a relatively low melting point and being (a) cast in a shape having an external profile which is undersized in a predetermined manner relative to the required external profile of the inductor, or (b) subsequently reduced in size so as to provide this undersized external profile; .
electrodepositing a thick metallic coating on the undersized external profile of the blank so as to provide a composite structure having an external profile which corresponds, or which is subsequently worked so as to correspond with the required external profile of the inductor, the coating being made of a material having a significantly higher melting point than that of the cast material forming the blank and being of sufficient thickness to provide a rigid structure upon subsequent removal of the material forming the blank; and
heating the cast material to liquid form and removing the liquid cast material, thereby forming the hollow inductor with the required external profile.

The method according to the further aspect of the invention is particularly useful in making a hollow inductor for use in induction hardening of gear teeth to provide surface hardening of the working surfaces of the gear teeth, and also to a significant depth below the surface, in which the inductor is caused to traverse along the gap defined between each pair of adjacent teeth during the induction hardening process. An inductor made by the method according to the further aspect of the invention can have its external profile made to accurate requirements concerning clearances between the external profile of the inductor and the flank and root surfaces of the gear teeth, which is one of a number of important parameters to be carefully controlled, to achieve satisfactory surface hardening, as taught by the disclosure in GB specification No. 2 143 854A.

When the method is used to make an inductor for surface hardening gear teeth, conveniently, though not essentially, the blank is cast in situ in the gap defined between a typical pair of adjacent gear teeth of the gear which is to be induction hardened. Preferably, the material from which the blank is cast is an alloy having a melting point in the range 70 to 80°C, so that the cast material can readily be removed from the composite structure - (formed by application of the metallic coating thereon) by the use of very hot water.

One preferred method of making a hollow inductor for use in induction hardening machines comprises the following steps:
1. Forming a blank of the profile of the component in/around which the inductor is required to fit, the blank being cast from a substance with a relatively low melting point, and the substance being electrically conductive when in the solid form;
2. The solidified blank is removed from the component;
3. Surface material is removed from the cast blank selectively in order to provide a required level of undersize on all/some selected surfaces or areas of the blank to provide an undersized blank;
4. The undersized blank is electroplated with a coating of metal or metals and/or alloy or alloys, to provide a thick, mechanically strong coating;
5. At least part of the surface of the thick mechanically strong coating is removed selectively to provide a smooth, uniform surface to required dimensions; and
6. The cast material forming the blank is removed from the composite structure of blank and coating, by the gentle application of heat, whereby the cast material melts and is poured, or otherwise removed, from inside the coating, leaving a mechanically strong shell of the required dimensions, to be assembled into an inductor for use in induction hardening of the surface of the component.

Additionally, the working surface of the component which is to be treated by the inductor may be covered with a lining, prior to casting of the blank therein, to reduce the amount of cast material which has to be removed to form the undersized blank.

Preferably, the lining is of variable thickness and/or held out of contact with the working surfaces of the component, to further reduce the amount of cast material which has to be removed from the blank in the formation of the undersized blank.

The material from which the blank is cast is an alloy having a melting point in the range of 70 to 80°C in the preferred method referred to above, and conveniently an alloy based on the metal bismuth may be used. Alloys with a melting point in the range of 70 to 80°C will be molten in very hot water, thereby facilitating the subsequent removal of the cast material from the composite structure.

In the formation of an inductor by a method according to the invention, it is preferred that the blank is electroplated with a metallic coating of copper or copper/nickel alloy. The electroplating may be done in alternating layers of copper and copper/nickel to improve the electrical and/or mechanical properties.

Further, it will be evident that the blank which is actually electroplated may be composed of more than one blank which has been cast and/or otherwise produced separately, and subsequently joined together in an electrically conductive manner. Furthermore, sections of the blank may be removed, to produce the required shape of blank which is to be electroplated.

The invention will nwo be described in more detail, by way of example only, with reference to the accompanying drawings in which:
Figure 1 is a perspective illustration of an inductor and connector block assembly for mounting in an induction heating head, the inductor being a typical example of a hollow working tool which can be made by a method according to the invention;
Figure 2 is a perspective view of the assembly of the inductor, and prior to the fitting of a magnetic intensifier therein;
Figure 3 is a sectional elevation showing the required clearances between the external profile of the inductor and the adjacent working surfaces of a pair of gear teeth which are to undergo induction hardening;
Figure 4 is a sectional elevation of a first stage of a method according to the invention for making the inductor shown in Figures 1 to 3;
Figure 5 is a sectional elevation, similar to Figure 4, illustrating an alternative first method stage;
Figure 6 is a sectional elevation, similar to Figure 5, illustrating a further alternative way of carrying out the first stage; and
Figure 7 illustrates an alloy blank formed by any of the first method stages shown in Figures 4 to 6, prior to electroplating of a metallic coating thereon.

In Figures 1 to 3, there is shown an inductor which is suitable for use in the induction hardening method and apparatus which is disclosed in more detail in our published GB specification No. 2 143 854A. Figures 1 to 3 have already been described in more detail in the introduction to this specification.

A method according to the invention, for making the inductor shown in Figures 1 to 3, will now be described in more detail with reference to Figures 4 to 7 of the accompanying drawings. To form the inductor 1, there is first formed, by casting, a solid blank which has an external profile which corresponds generally with the required external profile of the inductor, the blank being (a) cast in a shape having an external provile which is undersized in a predetermined manner relative to the required external profile of the inductor or (b) subsequently reduced in size so as to provide this undersized external profile. Following the formation of the cast solid blank with the undersized external profile, a thick metallic coating is applied so as to provide a composite structure having an external profile which corresponds, or which is subsequently worked so as to correspond with the required external profile of the inductor. The coating is made of a material having a significantly higher melting point that that of the cast solid blank, and is of sufficient thickness to provide a rigid structure, upon subsequent removal of the material forming the cast blank. Thereafter, the cast material is heated to liquid form and then is removed from the composite structure, thereby forming the hollow inductor with the required external profile.

Referring to Figure 4, there is shown the formation of a cast solid alloy blank B in the tooth space defined between a pair of adjacent gear teeth 10 of a gear which is to be induction hardened. The blank B is cast in a low melting point alloy, and a range of low melting point alloys is well known, the exact melting point being determined by varying the proportions of the alloying constituents. For the present application, an alloy having a melting point of 70 to 80° is ideal, and alloys having melting points in this range are frequently based on the metal bismuth. An alloy with a melting point in this range will be molten in very hot water.

The blank B with a profile of the gear tooth space can be obtained by placing blanking plates at each end of the tooth space, and filling the casting mould formed thereby with a molten alloy of the type referred to above. Figure 4 is a sectional elevation of the results achieved by this casting process. It is not necessary to use a space on the actual gear to form the casting mould. Frequently, "test arcs" of teeth are machined in order to ascertain the exact parameters for hardening, prior to hardening the actual gear wheel. One of the spaces on a test arc could readily be used instead, to form the required casting mould. Alternatively, a piece of another material, e. g. a non-metallic substance, such as Tufnol (Registered Trade Mark) could be specially prepared on the gear cutting machine to give the required profile, for use as the casting mould. It may be appropriately undersized, if required.

Once the alloy has solidified, the blank B is removed from the gear tooth space. It is probable that differential contraction on cooling will break the bond between alloy and gear teeth, but if this is not the case, a gentle tap on the end of the blank should serve equally well. Surface treatment of the gear teeth, e. g. polish, grease, etc. may also be used to facilitate the removal of the blank.

Having obtained the blank B the section - (Figure 4) must be reduced in size, initially by the removal of the thick layer equivalent to the required clearance (as shown in Figure 3), but then further by a suitable amount to allow for subsequent electroplating. A variety of methods may be used for reducing the blank in size, some of which are as follows:-
i) Mechanical methods, e. g. machining, filing, grinding, buffing, etc.
ii) Chemical methods, e. g. dissolution in acids, etc.
iii) Electrical methods, e. g. spark erosion, etc.
iv) Electrochemical methods, e. g. dissolution in an electrolyte.
v) Thermal methods, e.g. 'painting' the surface with a brush dipped in boiling water.

To achieve the required final dimensions one, or more, of the above methods may be used.

In order to reduce the volume of alloy to be removed, either or both of the following approaches may be adopted, i.e.
i) cast the alloy before final machining (prior to induction hardening) of the gear space is complete, or
ii) line the space so that the alloy does not actually contact the metal of the gear teeth

The casting may be performed at an intermediate stage in the machining process. By choosing the optimum stage in the machining process for casting, the volume of alloy which must subsequently be removed may be reduced to a minimum.

Thus, the tooth space 11 of an essentially finished machined gear may be lined with a lining membrane 12, as shown in Figure 5. The lining 12 may be metallic, e.g. an annealed copper sheet bent, and gently worked to the profile of the gear teeth 10. To allow for the changing clearances between inductor 1 and gear teeth 10 (Figure 2), lining 12 may be moved away from the addendum of gear teeth 10, e.g. by wedges 13 as shown in Figure 6. Non-metallic linings 12 could also be used. The thickness of lining 12 would be such as to minimise subsequent alloy-removal from the blank.

When the alloy has solidified and been removed from the gear space, it will be reduced in size, if necessary, to the final dimensions by one, or more of the methods previously outlined. the advantages of casting the alloy along the full width of a gear tooth are that several blanks makes it easier to hold during machining operations. One method of alloy removal after casting could be:-
i) machine full length of blank to required dimensions.
ii) mark positions of magnetic intensifier cut outs and remove unwanted metal.
iii) mark positions of pipes, and drill holes.
iv) cut the blank into individual lengths.

Separately from this work, undersized rods will be cast from the same alloy. The rods will be cast in an 'H' section (20, Figure 7), using conventional techniques, i.e. running liquid alloy into a hot mould, allowing to cool and separating the two halves of the mould to remove the casting.

When the individual alloy blanks have been prepared according to the sequence above, the H-shaped rod assembly 20 may be fitted by pushing the ends of the rods into the holes previously drilled in the blanks. The rods are then secured into the holes by careful use of a cool brazing torch. Alternatively, an artist's paint brush, dipped in boiling water and then applied to the joint may well create sufficient local heating to fuse the two components. Figure 7 shows the completed alloy blank. The cut out 22 is for subsequent insertion of the magnetic intensifier 2 (Figure 1).

The completed alloy block (Figure 7) is now placed in a bath of electrolyte and plated with copper. A chemical etching is sometimes used before electroplating to clean the alloy surfce and so encourage deposition of a uniformly thick layer. As the blank is a metallic alloy it will be electrically conducting. The cross bar on the H-shaped rod assembly 20 serves two functions. They are firstly to provide rigidity to the two vertical rods and secondly to improve the flow of electrical current over the blank so that a more uniform deposition takes place. Because the alloy block is an irregular shape, various known techniques may be adopted to obtain a coating of as uniform a thickness as possible. Such techniques could include the use of multiple anodes, agitation of the electrolyte, special, additives in the electrolyte, specially chosen current densities, etc.

After a suitable period of electroplating, an adequate thickness of copper and/or other metal(s) or alloys(s) will have been deposited. Then the block is removed from the electrolyte, washed and checked dimensionally. The copper surface of the inductor is now smoothed to remove 'high points' and give the final dimensions. This operation would probably be done carefully by a craftsman using a file or scraper; however, as the copper surface is well supported, careful handling on, for example a grinding wheel, may be possible. Once the sides of the cut-out have been smoothed, the magnetic intensifier (2) may be fitted and smoothed to the final dimensions at the same time as the rest of the inductor.

When final dimensions are achieved, the H-shaped rods 20 are cut-off along the plane AA. The component is now placed in boiling water and allowed to thoroughly heat through. When the alloy has melted, it may be run out via one of the copper pipes which have formed around the H-shaped rods 20. It is possible that gentle air or water pressure may have to be applied to one copper pipe, in order to cause the molten alloy to run out of the other. Once the inductor is free of alloy, it will be pressure tested to check for leaks and dimensionally checked. It will then be incorporated into the complete inductor assembly, as shown in Figure 1.

The advantage of the method disclosed herein is that inductors may be more easily, cheaply and accurately manufactured than by the existing fabrication techniques. For example, inductors for helically cut teeth could be made as easily as those for cross-cut teeth, whereas the fabrication method would be much more complex for helically cut teeth. Also smaller inductors could be made with the fabrication method, so extending downwards the size range of gears which can be hardened by the method and apparatus disclosed in our GB specification No. 2 143 854A.

While it is preferred that the cast blank B is made of electrically conductive material, to enable the subsequent application of the metallic coating thereon by electrodeposition, this is not essential to the invention. Other electrically conductive casting materials may be used, such as speciallised electrically conductive plastics material. Alternatively, non-conductive cast materials may be used, such as waxes and polymers, provided that an electrically conductive film is applied thereon, to form a cathode surface on which the electrodeposited metallic coating may be applied.

## Claims

A method of making a hollow working tool (1) for the treatment of a predetermined portion (10,11) of a workpiece, the tool having a predetermined external profile which corresponds generally with the shaped portion of the workpiece which is to be treated by the working tool, and the method comprising:
casting a solid blank (B) which has an external profile which corresponds generally with the required external profile of the tool, the blank being - (a) cast in a shape having an external profile which is undersized in a predetermined manner relative to the required external profile of the tool or (b) subsequently reduced insize so as to provide this undersized external profile;
applying a thick metallic coating to the undersized external profile of the blank so as to provide a composite sructure having an external profile which correpsonds, or which is subsequently worked so as to correspond with the required external profile of the tool, the coating being of sufficient thickness to provide a rigid structure upon subsequent removal of the material forming the cast blank ; and
removing the cast material from the composite structure, thereby forming the hollow working tool with the required external profile.

2. A method according to claim 1, in whichthe coating is made of a material having a significantly higher melting point than that of the cast solid blank, and the cast material is removed from the composite structure by the applciation of sufficient heat to melt the cast material which is then poured out of the composite structure.

3. A method according to claim 1, in which the cast material is removed from the composite structure by chemical means.

4. A method according to any one of the preceeding claims in which the thick metallic coating is applied by electrodeposition.

5. A method according to any one of the preceeding claims, in which the cast material which forms the blank is metallic.

6. A method according to any one of the preceeding claims, in which the blank is made of electrically conductive plastic material.

7. A method according to any one of the preceeding claims, in which the blank is made of non-conductive material, and a conductive film is applied to the external surface of the non-conductive material so as to promote electrodeposition of the coating thereon.

8. A method according to any one of the preceeding claims, in which the hollow working tool comprises a hollow inductor for use in an induction hardening machine.

9. A method of making a hollow inductor (1) for use in inductive heat treatment of a predetermined shaped portion (10,11) of a workpiece, by traversing the inductor along the surface of the shaped portion, the inductor having an external profile which corresponds generally with the shaped portion of the workpiece, and the method comprising:
casting a solid blank (B) which has an external profile which corresponds generally with the required external profile of the inductor, the blank being made of an electrically conductive material having a relatively low melting point and being (1) cast in a shape having an external profile which is undersized in a predetermined manner relative to the required external profile of the inductor, or (b) subsequently reduced in size so as to provide this undersized external profile;
electrodepositing a thick metallic coating on the undersized external profile of the blank so as to provide a composite structure having an external profile which corresponds, or which is subsequently worked so as to correspond with the required external profile of the inductor, the coating being made of a material having a significantly higher melting point than that of the cast material forming the blank and being of sufficient thickness to provide a rigid structure upon subsequent removal of the material forming the blank; and
heating the cast material to liquid form and removing the liquid cast material, thereby forming the hollow inductor with the required external profile.

10. A method according to claim 9, for making a hollow inductor intended for surface hardening of gear teeth, in which the blank is cast in situ in the gap (11) defined between a typical pair of adjacent gear teeth (10) of the gear which is to be induction hardened, or a model of a typical pair of adjacent gear teeth.

11. A method according to claims 9 or 10, in which the working surface of the component which is to be treated by the inductor is covered with a lining - (12), prior to the casting of the blank, to reduce the amount of cast material which has to be removed subsequently to form the undersized blank.

12. A method according to claim 11, in which the lining is of variable thickness and/or held out of contact with the working surface of the component, to further reduce the amount of cast material which has to be removed subsequently to form the blank.

13. A method according to claims 9 to 12, in which the blank is cast in an alloy having a melting point in the range 70° to 80°C.

14. A method according to claim 13, in which the alloy is based on bismuth.

15. A method according to any one of claims 9 to 14, in which the blank is electroplated with a metallic coating of copper or copper/nickel alloy.

16. A method according to claims 9 to 15, in which a cut-out (22) is formed in the composite structure, and a magnetic intensifier (2) is fited in said cut-out after removal of the cast material.
